



US009993692B2

(12) **United States Patent**  
**Isogawa et al.**

(10) **Patent No.:** **US 9,993,692 B2**  
(b4) **Date of Patent:** **\*Jun. 12, 2018**

(54) **GOLF BALL**(71) Applicant: **DUNLOP SPORTS CO. LTD.**,  
Kobe-shi, Hyogo (JP)(72) Inventors: **Kazuhiko Isogawa**, Kobe (JP); **Kosuke Tachibana**, Kobe (JP)(73) Assignee: **SUMITOMO RUBBER INDUSTRIES, LTD.**, Kobe-Shi, Hyogo (JP)

(\*) Notice: Subject to any disclaimer, the term of this patent is extended or adjusted under 35 U.S.C. 154(b) by 0 days. days.

This patent is subject to a terminal disclaimer.

(21) Appl. No.: **14/902,173**(22) PCT Filed: **Oct. 7, 2014**(86) PCT No.: **PCT/JP2014/076793**

§ 371 (c)(1),

(2) Date: **Dec. 30, 2015**(87) PCT Pub. No.: **WO2015/053259**PCT Pub. Date: **Apr. 16, 2015**(65) **Prior Publication Data**

US 2016/0367864 A1 Dec. 22, 2016

(30) **Foreign Application Priority Data**

Oct. 8, 2013 (JP) ..... 2013-210823

(51) **Int. Cl.****A63B 37/00** (2006.01)(52) **U.S. Cl.**CPC ..... **A63B 37/0092** (2013.01); **A63B 37/004** (2013.01); **A63B 37/008** (2013.01);

(Continued)

(58) **Field of Classification Search**CPC ..... A63B 37/0031; A63B 37/0033; A63B 37/0043; A63B 37/0045; A63B 37/0063;  
(Continued)(56) **References Cited**

## U.S. PATENT DOCUMENTS

6,152,834 A \* 11/2000 Sullivan ..... A63B 37/0003  
473/365  
2004/0235587 A1 \* 11/2004 Sullivan ..... A63B 37/008  
473/371

(Continued)

## FOREIGN PATENT DOCUMENTS

JP 2007-319660 A 12/2007  
JP 2007-319667 A 12/2007  
(Continued)

## OTHER PUBLICATIONS

International Search Report issued in PCT/JP2014/076793 dated Jan. 6, 2015.

(Continued)

*Primary Examiner* — John E Simms, Jr.(74) *Attorney, Agent, or Firm* — Birch, Stewart, Kolasch & Birch, LLP(57) **ABSTRACT**

A golf ball includes a spherical core, a mid layer, an inner cover, and an outer cover. A hardness  $H_m$  of the mid layer is greater than a hardness  $H_{inc}$  of the inner cover which is greater than a hardness  $H_{ouc}$  of the outer cover. A difference  $(H_m - H_{ouc})$  is greater than 25. A volume  $V_m$  of the mid layer is greater than a volume  $V_{inc}$  of the inner cover which is greater than a volume  $V_{ouc}$  of the outer cover. A ratio  $[(V_m + V_{inc} + V_{ouc})/V]$  of a sum  $(V_m + V_{inc} + V_{ouc})$  relative to a volume  $V$  of an entirety of the golf ball is less than 0.30. A ratio  $(V_m/V_{ouc})$  is greater than 1.50. A product  $(V_m * H_m)$  and a product  $(V_{ouc} * H_{ouc})$  meet the following relationship:  $[(V_m * H_m) / (V_{ouc} * H_{ouc})] > 3.0$ .

**17 Claims, 1 Drawing Sheet**

|                                                                |                                                                                                                                                                                                                                                                                                                                                                                                                                                  |                                                                                                          |
|----------------------------------------------------------------|--------------------------------------------------------------------------------------------------------------------------------------------------------------------------------------------------------------------------------------------------------------------------------------------------------------------------------------------------------------------------------------------------------------------------------------------------|----------------------------------------------------------------------------------------------------------|
| (52) <b>U.S. Cl.</b>                                           |                                                                                                                                                                                                                                                                                                                                                                                                                                                  | 2010/0075778 A1* 3/2010 Kamino ..... A63B 37/0003<br>473/376                                             |
| CPC .....                                                      | <i>A63B 37/0031</i> (2013.01); <i>A63B 37/0033</i> (2013.01); <i>A63B 37/0039</i> (2013.01); <i>A63B 37/0043</i> (2013.01); <i>A63B 37/0044</i> (2013.01); <i>A63B 37/0045</i> (2013.01); <i>A63B 37/0051</i> (2013.01); <i>A63B 37/0063</i> (2013.01); <i>A63B 37/0064</i> (2013.01); <i>A63B 37/0076</i> (2013.01); <i>A63B 37/0083</i> (2013.01); <i>A63B 37/0087</i> (2013.01); <i>A63B 37/0094</i> (2013.01); <i>A63B 37/0096</i> (2013.01) | 2011/0092315 A1* 4/2011 Nakamura ..... A63B 37/0031<br>473/376                                           |
|                                                                |                                                                                                                                                                                                                                                                                                                                                                                                                                                  | 2011/0300968 A1* 12/2011 Ryu ..... A63B 37/0043<br>473/373                                               |
|                                                                |                                                                                                                                                                                                                                                                                                                                                                                                                                                  | 2012/0214613 A1 8/2012 Okabe et al.                                                                      |
|                                                                |                                                                                                                                                                                                                                                                                                                                                                                                                                                  | 2013/0005508 A1 1/2013 Matsuyama et al.                                                                  |
|                                                                |                                                                                                                                                                                                                                                                                                                                                                                                                                                  | 2013/0065707 A1* 3/2013 Matsuyama ..... C08K 5/09<br>473/373                                             |
| (58) <b>Field of Classification Search</b>                     |                                                                                                                                                                                                                                                                                                                                                                                                                                                  | FOREIGN PATENT DOCUMENTS                                                                                 |
| CPC .....                                                      | A63B 37/0064; A63B 37/0076; A63B 37/0092                                                                                                                                                                                                                                                                                                                                                                                                         | JP 2008-068077 A 3/2008                                                                                  |
| See application file for complete search history.              |                                                                                                                                                                                                                                                                                                                                                                                                                                                  | JP 2008-149130 A 7/2008                                                                                  |
| (56) <b>References Cited</b>                                   |                                                                                                                                                                                                                                                                                                                                                                                                                                                  | JP 2009-254471 A 11/2009                                                                                 |
| U.S. PATENT DOCUMENTS                                          |                                                                                                                                                                                                                                                                                                                                                                                                                                                  | JP 2010-068997 A 4/2010                                                                                  |
| 2007/0281801 A1 12/2007 Watanabe et al.                        |                                                                                                                                                                                                                                                                                                                                                                                                                                                  | JP 2010-099436 A 5/2010                                                                                  |
| 2008/0064526 A1 3/2008 Watanabe et al.                         |                                                                                                                                                                                                                                                                                                                                                                                                                                                  | JP 2011-083395 A 4/2011                                                                                  |
| 2008/0146377 A1* 6/2008 Watanabe ..... A63B 37/0031<br>473/376 |                                                                                                                                                                                                                                                                                                                                                                                                                                                  | JP 2011-255172 A 12/2011                                                                                 |
| 2009/0258731 A1* 10/2009 Kamino ..... A63B 37/0003<br>473/376  |                                                                                                                                                                                                                                                                                                                                                                                                                                                  | JP 2012-170629 A 9/2012                                                                                  |
| 2010/0069175 A1* 3/2010 Kamino ..... A63B 37/0003<br>473/376   |                                                                                                                                                                                                                                                                                                                                                                                                                                                  | JP 2013-056013 A 3/2013                                                                                  |
|                                                                |                                                                                                                                                                                                                                                                                                                                                                                                                                                  | OTHER PUBLICATIONS                                                                                       |
|                                                                |                                                                                                                                                                                                                                                                                                                                                                                                                                                  | Written Opinion of the International Searching Authority issued in PCT/JP2014/076793 dated Jan. 6, 2015. |

\* cited by examiner



**1**  
**GOLF BALL**

TECHNICAL FIELD

The present invention relates to golf balls. Specifically, the present invention relates to golf balls that include a core, a mid layer, an inner cover, and an outer cover.

BACKGROUND ART

Golf players' foremost requirement for golf balls is high flight distance performance. In particular, golf players place importance on high flight distance performance upon a shot with a driver. High flight distance performance correlates with the resilience performance of a golf ball. When a golf ball having excellent resilience performance is hit, the golf ball flies at a high speed, thereby achieving a large flight distance.

An appropriate trajectory height is required in order to achieve a large flight distance. A trajectory height depends on a spin rate and a launch angle. With a golf ball that achieves a high trajectory by a high spin rate, a flight distance is insufficient. With a golf ball that achieves a high trajectory by a high launch angle, a large flight distance is obtained. Use of a core having an outer-hard/inner-soft structure can achieve a low spin rate and a high launch angle.

Golf players also place importance on spin performance of golf balls. When a backspin rate is high, the run is short. It is easy for golf players to cause a golf ball, to which backspin is easily provided, to stop at a target point. When a sidespin rate is high, the golf ball tends to curve. It is easy for golf players to intentionally cause a golf ball, to which sidespin is easily provided, to curve. A golf ball to which spin is easily provided has excellent approach performance. In particular, advanced golf players place importance on approach performance upon a shot with a short iron.

Golf players are further interested in feel at impact of golf balls. A hard cover deteriorates feel at impact. Golf players prefer soft feel at impact.

In light of achievement of various performance characteristics, golf balls each having a multilayer structure have been proposed. Japanese Patent Application Laid-Open No. 2007-319660 discloses a golf ball that includes a core, an envelope layer, a mid layer, and a cover. The mid layer of the golf ball is harder than the envelope layer and the cover thereof. Japanese Patent Application Laid-Open No. 2007-319667 and Japanese Patent Application Laid-Open No. 2008-68077 also disclose similar golf balls. Japanese Patent Application Laid-Open No. 2011-255172 discloses a golf ball that includes a central portion, a mid layer, and an outer layer. The outer layer of the golf ball is relatively hard and thick. U.S. Pat. No. 6,152,834 discloses a golf ball that includes a core and a cover having at least three layers. In the golf ball, a soft and thick cover is formed as an outermost layer.

CITATION LIST

Patent Literature

Patent Literature 1: Japanese Patent Application Laid-Open No. 2007-319660

Patent Literature 2: Japanese Patent Application Laid-Open No. 2007-319667

Patent Literature 3: Japanese Patent Application Laid-Open No. 2008-68077

**2**

Patent Literature 4: Japanese Patent Application Laid-Open No. 2011-255172

Patent Literature 5: U.S. Pat. No. 6,152,834

SUMMARY OF INVENTION

Technical Problem

When a golf ball having a high launch angle and a low spin rate is hit with a driver, a large flight distance is obtained. However, a golf ball having a low spin rate has inferior approach performance. In recently years, golf players' requirements for golf balls have been escalated more than ever. A golf ball that achieves both a large flight distance and excellent approach performance on a high level is desired. Furthermore, a golf ball having soft feel at impact upon a shot is desired.

An object of the present invention is to provide a golf ball that has high flight distance performance upon a shot with a driver and excellent approach performance upon a shot with a short iron and provides favorable feel at impact.

Solution to Problem

A golf ball according to the present invention includes a spherical core, a mid layer positioned outside the core, an inner cover positioned outside the mid layer, and an outer cover positioned outside the inner cover. In the golf ball, a Shore D hardness  $H_m$  of the mid layer is greater than a Shore D hardness  $H_{inc}$  of the inner cover, and the hardness  $H_{inc}$  is greater than a Shore D hardness  $H_{ouc}$  of the outer cover. A difference ( $H_m - H_{ouc}$ ) between the hardness  $H_m$  and the hardness  $H_{ouc}$  is greater than 25. In the golf ball, a volume  $V_m$  of the mid layer is greater than a volume  $V_{inc}$  of the inner cover, and the volume  $V_{inc}$  is greater than a volume  $V_{ouc}$  of the outer cover. A ratio  $[(V_m + V_{inc} + V_{ouc})/V]$  of a sum  $(V_m + V_{inc} + V_{ouc})$  of the volume  $V_m$ , the volume  $V_{inc}$ , and the volume  $V_{ouc}$  relative to a volume  $V$  of an entirety of the golf ball is less than 0.30. A ratio  $(V_m/V_{ouc})$  of the volume  $V_m$  relative to the volume  $V_{ouc}$  is greater than 1.50. A product  $(V_m * H_m)$  of the hardness  $H_m$  and the volume  $V_m$  and a product  $(V_{ouc} * H_{ouc})$  of the hardness  $H_{ouc}$  and the volume  $V_{ouc}$  meet the following relationship.

$$[(V_m * H_m) / (V_{ouc} * H_{ouc})] > 3.0$$

Preferably, a ratio  $(V_{ouc}/V)$  of the volume  $V_{ouc}$  relative to the volume  $V$  is less than 0.08.

The hardness  $H_{ouc}$  is preferably equal to or less than 36.

Preferably, the mid layer is formed from a resin composition. A principal component of a base resin of the resin composition is preferably selected from an ionomer resin, a polyamide resin, and a mixture thereof.

The hardness  $H_m$  is preferably equal to or greater than 68.

Preferably, a JIS-C hardness  $H_s$  at a surface of the core is greater than a JIS-C hardness  $H_o$  at a central point of the core. A difference ( $H_s - H_o$ ) between the hardness  $H_s$  and the hardness  $H_o$  is preferably equal to or greater than 20.

Preferably, the core is obtained by a rubber composition being crosslinked. Preferably, the rubber composition includes a fatty acid or a fatty acid metal salt.

Advantageous Effects of Invention

The golf ball according to the present invention includes the mid layer, the inner cover, and the outer cover on the external side of the core. The hardness of each layer is decreased in order from the outside of the core toward the

ball surface. In the golf ball, the volume of each layer is set in an appropriate range. When the golf ball is hit with a short iron, the spin rate is high. The golf ball has excellent approach performance. In the golf ball, the resilience performance of the core is not impaired. When the golf ball is hit with a driver, the spin rate is low. The excellent resilience performance and the low spin rate achieve a large flight distance. The feel at impact of the golf ball is soft.

#### BRIEF DESCRIPTION OF DRAWINGS

FIG. 1 is a partially cutaway cross-sectional view of a golf ball according to one embodiment of the present invention.

#### DESCRIPTION OF EMBODIMENTS

The following will describe in detail the present invention, based on preferred embodiments with reference to the accompanying drawing.

FIG. 1 is a partially cutaway cross-sectional view of a golf ball 2 according to one embodiment of the present invention. The golf ball 2 includes a spherical core 4, an inner cover 8 positioned outside the core 4, an inner cover 8 positioned outside the mid layer 6, a reinforcing layer 10 positioned outside the inner cover 8, and an outer cover 12 positioned outside the reinforcing layer 10. On the surface of the outer cover 12, a large number of dimples 14 are formed. Of the surface of the outer cover 12, a part other than the dimples 14 is a land 16. The golf ball 2 includes a paint layer and a mark layer on the external side of the outer cover 12, but these layers are not shown in the drawing.

The golf ball 2 has a diameter of 40 mm or greater but 45 mm or less. From the standpoint of conformity to the rules established by the United States Golf Association (USGA), the diameter is preferably equal to or greater than 42.67 mm. In light of suppression of air resistance, the diameter is preferably equal to or less than 44 mm and more preferably equal to or less than 42.80 mm. The golf ball 2 has a weight of 40 g or greater but 50 g or less. In light of attainment of great inertia, the weight is preferably equal to or greater than 44 g and more preferably equal to or greater than 45.00 g. From the standpoint of conformity to the rules established by the USGA, the weight is preferably equal to or less than 45.93 g.

Preferably, the core 4 is obtained by crosslinking a rubber composition. Examples of preferable base rubbers for use in the rubber composition include polybutadienes, polyisoprenes, styrene-butadiene copolymers, ethylene-propylene-diene copolymers, and natural rubbers. In light of resilience performance, polybutadienes are preferred. When a polybutadiene and another rubber are used in combination, it is preferred if the polybutadiene is included as a principal component. Specifically, the proportion of the polybutadiene to the entire base rubber is preferably equal to or greater than 50% by weight and more preferably equal to or greater than 80% by weight. The proportion of cis-1,4 bonds in the polybutadiene is preferably equal to or greater than 40% and more preferably equal to or greater than 80%.

The rubber composition of the core 4 includes a co-crosslinking agent. The co-crosslinking agent achieves high resilience performance of the core 4. Examples of preferable co-crosslinking agents in light of resilience performance include monovalent or bivalent metal salts of an  $\alpha,\beta$ -unsaturated carboxylic acid having 2 to 8 carbon atoms. A metal salt of an  $\alpha,\beta$ -unsaturated carboxylic acid graft-polymerizes with the molecular chain of the base rubber, thereby crosslinking the rubber molecules. Specific

examples of preferable co-crosslinking agents include zinc acrylate, magnesium acrylate, zinc methacrylate, and magnesium methacrylate. Zinc acrylate and zinc methacrylate are particularly preferred on the grounds that high resilience performance is achieved.

As a co-crosslinking agent, an  $\alpha,\beta$ -unsaturated carboxylic acid having 2 to 8 carbon atoms and a metal compound may also be included. The metal compound reacts with the  $\alpha,\beta$ -unsaturated carboxylic acid in the rubber composition.

- 10 A salt obtained by this reaction graft-polymerizes with the molecular chain of the base rubber. Examples of preferable  $\alpha,\beta$ -unsaturated carboxylic acids include acrylic acid and methacrylic acid.

Examples of preferable metal compounds include metal hydroxides such as magnesium hydroxide, zinc hydroxide, calcium hydroxide, and sodium hydroxide; metal oxides such as magnesium oxide, calcium oxide, zinc oxide, and copper oxide; and metal carbonates such as magnesium carbonate, zinc carbonate, calcium carbonate, sodium carbonate, lithium carbonate, and potassium carbonate. Metal oxides are preferred. Oxides including a bivalent metal are more preferred. An oxide including a bivalent metal reacts with the co-crosslinking agent to form metal crosslinks. Examples of particularly preferable metal oxides include zinc oxide and magnesium oxide.

In light of resilience performance of the golf ball 2, the amount of the co-crosslinking agent per 100 parts by weight of the base rubber is preferably equal to or greater than 25 parts by weight and more preferably equal to or greater than 30 parts by weight. In light of soft feel at impact, the amount of the co-crosslinking agent per 100 parts by weight of the base rubber is preferably equal to or less than 50 parts by weight and more preferably equal to or less than 45 parts by weight.

35 Preferably, the rubber composition of the core 4 includes an organic peroxide together with the co-crosslinking agent. The organic peroxide serves as a crosslinking initiator. The organic peroxide contributes to the resilience performance of the golf ball 2. Examples of suitable organic peroxides include dicumyl peroxide, 1,1-bis(t-butylperoxy)-3,3,5-trimethylcyclohexane, 2,5-dimethyl-2,5-di(t-butylperoxy)hexane, and di-t-butyl peroxide. In light of versatility, dicumyl peroxide is preferred.

In light of resilience performance of the golf ball 2, the amount of the organic peroxide per 100 parts by weight of the base rubber is preferably equal to or greater than 0.1 parts by weight, more preferably equal to or greater than 0.3 parts by weight, and particularly preferably equal to or greater than 0.5 parts by weight. In light of soft feel at impact, the amount of the organic peroxide per 100 parts by weight of the base rubber is preferably equal to or less than 2.0 parts by weight, more preferably equal to or less than 1.5 parts by weight, and particularly preferably equal to or less than 1.2 parts by weight.

55 Preferably, the rubber composition of the core 4 includes an organic sulfur compound. Examples of preferable organic sulfur compounds include monosubstitutions such as diphenyl disulfide, bis(4-chlorophenyl)disulfide, bis(3-chlorophenyl)disulfide, bis(4-bromophenyl)disulfide, bis(3-bromophenyl)disulfide, bis(4-fluorophenyl)disulfide, bis(4-iodophenyl)disulfide, bis(4-cyanophenyl)disulfide, and the like; disubstitutions such as bis(2,5-dichlorophenyl)disulfide, bis(3,5-dichlorophenyl)disulfide, bis(2,6-dichlorophenyl)disulfide, bis(2,5-dibromophenyl)disulfide, bis(3,5-dibromophenyl)disulfide, bis(2-chloro-5-bromophenyl)disulfide, bis(2-cyano-5-bromophenyl)disulfide, and the like; trisubstitutions such as bis(2,4,6-trichlorophenyl)disulfide.

fide, bis(2-cyano-4-chloro-6-bromophenyl)disulfide, and the like; tetrasubstitutions such as bis(2,3,5,6-tetrachlorophenyl)disulfide and the like; and pentasubstitutions such as bis(2,3,4,5,6-pentachlorophenyl)disulfide, bis(2,3,4,5,6-pentabromophenyl)disulfide, and the like. Other examples of preferable organic sulfur compounds include thionaphthols such as 2-thionaphthol, 1-thionaphthol, 2-chloro-1-thionaphthol, 2-bromo-1-thionaphthol, 2-fluoro-1-thionaphthol, 2-cyano-1-thionaphthol, 2-acetyl-1-thionaphthol, 1-chloro-2-thionaphthol, 1-bromo-2-thionaphthol, 1-fluoro-2-thionaphthol, 1-cyano-2-thionaphthol, 1-acetyl-2-thionaphthol, and the like; and metal salts thereof. The organic sulfur compound contributes to resilience performance. More preferable organic sulfur compounds are 2-thionaphthol, diphenyl disulfide, and bis(pentabromophenyl)disulfide. A particularly preferable organic sulfur compound is 2-thionaphthol.

In light of resilience performance of the golf ball **2**, the amount of the organic sulfur compound per 100 parts by weight of the base rubber is preferably equal to or greater than 0.10 parts by weight, more preferably equal to or greater than 0.15 parts by weight, and particularly preferably equal to or greater than 0.20 parts by weight. In light of resilience performance, the amount is preferably equal to or less than 5.0 parts by weight, more preferably equal to or less than 3.0 parts by weight, and particularly preferably equal to or less than 1.0 parts by weight.

Preferably, the rubber composition of the core **4** further includes a fatty acid or a fatty acid metal salt. During heating and forming of the core **4**, the fatty acid dissociates and reacts with the cationic component of the co-crosslinking agent. It is thought that within the core **4**, the fatty acid inhibits formation of the metal crosslinks by the co-crosslinking agent. The acid component included in the fatty acid metal salt exchanges the cationic component with the co-crosslinking agent. It is inferred that during heating and forming of the core **4**, the fatty acid metal salt breaks the metal crosslinks by the co-crosslinking agent.

In light of reactivity with the co-crosslinking agent, the carbon number of the fatty acid component included in the fatty acid or the fatty acid metal salt is preferably equal to or greater than 4. In light of mixability with the other components in the rubber composition, the carbon number of the fatty acid component is preferably equal to or less than 30, more preferably equal to or less than 20, and particularly preferably equal to or less than 15.

Examples of fatty acids include butyric acid (C4), valeric acid (C5), caproic acid (C6), enanthic acid (C7), caprylic acid (octanoic acid) (C8), pelargonic acid (C9), capric acid (decanoic acid) (C10), lauric acid (C12), myristic acid (C14), myristoleic acid (C14), pentadecylic acid (C15), palmitic acid (C16), palmitoleic acid (C16), margaric acid (C17), stearic acid (C18), elaidic acid (C18), vaccenic acid (C18), oleic acid (C18), linolic acid (C18), linolenic acid (C18), 12-hydroxystearic acid (C18), arachidic acid (C20), gadoleic acid (C20), arachidonic acid (C20), eicosenoic acid (C20), behenic acid (C22), erucic acid (C22), lignoceric acid (C24), nervonic acid (C24), cerotic acid (C26), montanic acid (C28), and melissic acid (C30). Two or more fatty acids may be used in combination. Caprylic acid (octanoic acid), lauric acid, myristic acid, palmitic acid, stearic acid, oleic acid, and behenic acid are preferred.

The fatty acid metal salt includes a metal ion. Examples of the metal ion include sodium ion, potassium ion, lithium ion, silver ion, magnesium ion, calcium ion, zinc ion, barium ion, cadmium ion, copper ion, cobalt ion, nickel ion, man-

ganese ion, aluminum ion, iron ion, tin ion, zirconium ion, titanium ion, and the like. Two or more types of ions may be used in combination. Zinc ion and magnesium ion are preferred.

Examples of preferable fatty acid metal salts include potassium salts, magnesium salts, aluminum salts, zinc salts, iron salts, copper salts, nickel salts, and cobalt salts of octanoic acid, lauric acid, myristic acid, palmitic acid, stearic acid, oleic acid, and behenic acid. Zinc salts of fatty acids are particularly preferred. Specific examples of preferable zinc salts of fatty acids include zinc octoate, zinc laurate, zinc myristate, and zinc stearate. A fatty acid and a fatty acid metal salt may be used in combination, or two or more fatty acid metal salts may be used in combination.

In light of suppression of spin, the amount of the fatty acid or the fatty acid metal salt per 100 parts by weight of the base rubber is preferably equal to or greater than 0.5 parts by weight, more preferably equal to or greater than 1.0 parts by weight, and particularly preferably equal to or greater than 1.5 parts by weight. In light of resilience performance, the amount is preferably equal to or less than 20 parts by weight, more preferably equal to or less than 15 parts by weight, and particularly preferably equal to or less than 10 parts by weight.

As the co-crosslinking agent, zinc acrylate is preferably used. Zinc acrylate whose surface is coated with stearic acid or zinc stearate for the purpose of improving dispersibility to rubber is present. When the rubber composition includes this zinc acrylate, the stearic acid or zinc stearate coating the zinc acrylate is not included in the concept of the fatty acid or the fatty acid metal salt.

For the purpose of adjusting specific gravity and the like, a filler may be included in the core **4**. Examples of suitable fillers include zinc oxide, barium sulfate, calcium carbonate, and magnesium carbonate. Powder of a metal with a high specific gravity may be included as a filler. Specific examples of metals with a high specific gravity include tungsten and molybdenum. The amount of the filler is determined as appropriate so that the intended specific gravity of the core **4** is accomplished. A particularly preferable filler is zinc oxide. Zinc oxide serves not only as a specific gravity adjuster but also as a crosslinking activator. According to need, various additives such as sulfur, an anti-aging agent, a coloring agent, a plasticizer, a dispersant, and the like are included in the core **4** in an adequate amount. Crosslinked rubber powder or synthetic resin powder may also be included in the core **4**.

Preferably, a JIS-C hardness Ho at the central point of the core **4** is equal to or greater than 40 but equal to or less than 80. The core **4** having a hardness Ho of 40 or greater can achieve excellent resilience performance. In this respect, the hardness Ho is more preferably equal to or greater than 50 and particularly preferably equal to or greater than 55. The core **4** having a hardness Ho of 80 or less suppresses excessive spin upon a shot with a driver. In this respect, the hardness Ho is more preferably equal to or less than 76 and particularly preferably equal to or less than 72. The hardness Ho is measured by pressing a JIS-C type hardness scale against the central point of a cut plane of the core **4** that has been cut into two halves. For the measurement, an automated rubber hardness measurement machine (trade name "P1", manufactured by Kobunshi Keiki Co., Ltd.), to which this hardness scale is mounted, is used.

Preferably, a JIS-C hardness Hs at the surface of the core **4** is equal to or greater than 80 but equal to or less than 96. The core **4** having a hardness Hs of 80 or greater suppresses excessive spin upon a shot with a driver. In this respect, the

hardness Hs is more preferably equal to or greater than 82 and particularly preferably equal to or greater than 84. Due to the core **4** having a hardness Hs of 96 or less, excellent durability is obtained. In this respect, the hardness Hs is more preferably equal to or less than 94 and particularly preferably equal to or less than 92. The hardness Hs is measured by pressing a JIS-C type hardness scale against the surface of the core **4**. For the measurement, an automated rubber hardness measurement machine (trade name "P1", manufactured by Kobunshi Keiki Co., Ltd.), to which this hardness scale is mounted, is used.

Preferably, the hardness Hs is greater than the hardness Ho. In the core **4**, an outer-hard/inner-soft structure is formed. In the golf ball **2** including the core **4**, a spin rate is suppressed upon a shot with a driver. In this respect, the difference (Hs-Ho) between the hardness Hs and the hardness Ho is preferably equal to or greater than 20, more preferably equal to or greater than 23, and particularly preferably equal to or greater than 26. In light of resilience performance, the difference (Hs-Ho) is preferably equal to or less than 40 and more preferably equal to or less than 35.

In light of feel at impact, the core **4** has an amount of compressive deformation of preferably 2.0 mm or greater, more preferably 2.2 mm or greater, and particularly preferably 2.4 mm or greater. In light of resilience performance, the amount of compressive deformation is preferably equal to or less than 4.0 mm, more preferably equal to or less than 3.6 mm, and particularly preferably equal to or less than 3.4 mm.

In light of resilience performance, the core **4** has a diameter of preferably 37.0 mm or greater, more preferably 37.5 mm or greater, and particularly preferably 38.0 mm or greater. The diameter is preferably equal to or less than 42.0 mm, more preferably equal to or less than 41.0 mm, and particularly preferably equal to or less than 40.2 mm. The core **4** preferably has a weight of 25 g or greater but 42 g or less. The temperature for crosslinking the core **4** is generally equal to or higher than 140° C. but equal to or lower than 180° C. The time period for crosslinking the core **4** is generally equal to or longer than 10 minutes but equal to or shorter than 60 minutes. The core **4** may be formed with two or more layers.

For the mid layer **6**, a resin composition is suitably used. Examples of the base resin of the resin composition include ionomer resins, thermoplastic polyester elastomers, thermoplastic polyamide elastomers, thermoplastic polyurethane elastomers, thermoplastic polyolefin elastomers, and thermoplastic polystyrene elastomers.

The mid layer **6** may include a highly elastic resin. Examples of highly elastic resins include polyamide resins, polybutylene terephthalate, polyphenylene ether, polyethylene terephthalate, polysulfone, polyethersulfone, polyphenylene sulfide, polyarylate, polyamide imide, polyetherimide, polyether ether ketone, polyimide, polytetrafluoroethylene, polyamino bismaleimide, polybis-amide triazole, polyphenylene oxide, polyacetal, polycarbonate, acrylonitrile-butadiene-styrene copolymers, and acrylonitrile-styrene copolymers.

Preferable base resins in light of resilience performance are ionomer resins or polyamide resins. As described later, the cover of the golf ball **2** is thin. When the golf ball **2** is hit, the mid layer **6** significantly deforms due to the thinness of the cover. Ionomer resins and polyamide resins are highly elastic. The mid layer **6** including an ionomer resin or a polyamide resin contributes to resilience performance. An ionomer resin and a polyamide resin may be mixed and used.

Examples of preferable ionomer resins include binary copolymers formed with an  $\alpha$ -olefin and an  $\alpha,\beta$ -unsaturated carboxylic acid having 3 to 8 carbon atoms. A preferable binary copolymer includes 80% by weight or more but 90% by weight or less of an  $\alpha$ -olefin, and 10% by weight or more but 20% by weight or less of an  $\alpha,\beta$ -unsaturated carboxylic acid. The binary copolymer has excellent resilience performance. Examples of other preferable ionomer resins include ternary copolymers formed with: an  $\alpha$ -olefin; an  $\alpha,\beta$ -unsaturated carboxylic acid having 3 to 8 carbon atoms; and an  $\alpha,\beta$ -unsaturated carboxylate ester having 2 to 22 carbon atoms. A preferable ternary copolymer includes 70% by weight or more but 85% by weight or less of an  $\alpha$ -olefin, 5% by weight or more but 30% by weight or less of an  $\alpha,\beta$ -unsaturated carboxylic acid, and 1% by weight or more but 25% by weight or less of an  $\alpha,\beta$ -unsaturated carboxylate ester. The ternary copolymer has excellent resilience performance. For the binary copolymer and the ternary copolymer, preferable  $\alpha$ -olefins are ethylene and propylene, while preferable  $\alpha,\beta$ -unsaturated carboxylic acids are acrylic acid and methacrylic acid. A particularly preferable ionomer resin is a copolymer formed with ethylene and acrylic acid or methacrylic acid.

In the binary copolymer and the ternary copolymer, some of the carboxyl groups are neutralized with metal ions. Examples of metal ions for use in neutralization include sodium ion, potassium ion, lithium ion, zinc ion, calcium ion, magnesium ion, aluminum ion, and neodymium ion. The neutralization may be carried out with two or more types of metal ions. Particularly suitable metal ions in light of resilience performance and durability of the golf ball **2** are sodium ion, zinc ion, lithium ion, and magnesium ion.

Specific examples of ionomer resins include trade names "Himilan 1555", "Himilan 1557", "Himilan 1605", "Himilan 1706", "Himilan 1707", "Himilan 1856", "Himilan 1855", "Himilan AM7311", "Himilan AM7315", "Himilan AM7317", "Himilan AM7318", "Himilan AM7329", "Himilan MK7337", "Himilan MK7320", and "Himilan MK7329", manufactured by Du Pont-MITSUI POLY-CHEMICALS Co., Ltd.; trade names "Surlyn 6120", "Surlyn 6910", "Surlyn 7930", "Surlyn 7940", "Surlyn 8140", "Surlyn 8150", "Surlyn 8940", "Surlyn 8945", "Surlyn 9120", "Surlyn 9150", "Surlyn 9910", "Surlyn 9945", "Surlyn AD8546", "HPF1000", and "HPF2000", manufactured by E.I. du Pont de Nemours and Company; and trade names "IOTEK 7010", "IOTEK 7030", "IOTEK 7510", "IOTEK 7520", "IOTEK 8000", and "IOTEK 8030", manufactured by ExxonMobil Chemical Corporation. Two or more ionomer resins may be used in combination. An ionomer resin neutralized with a monovalent metal ion, and an ionomer resin neutralized with a bivalent metal ion may be used in combination.

A polyamide resin is a polymer having a plurality of amide bonds ( $-\text{NH}-\text{CO}-$ ) in the main chain thereof. Examples of polyamide resins include aliphatic polyamides, aromatic polyamides, amide copolymers, and the like. Examples of aliphatic polyamides include polyamide 6, polyamide 11, polyamide 12, polyamide 66, polyamide 610, polyamide 6T, polyamide 61, polyamide 9T, polyamide M5T, and polyamide 612. Examples of aromatic polyamides include poly-p-phenylene terephthalamide and poly-m-phenylene isophthalamide.

Examples of amide copolymers include polyether block amide copolymers, polyester amide copolymers, polyether ester amide copolymers, and polyamide imide copolymers. The polyamide resin may contain two or more polyamides. Aliphatic polyamides are preferred, and polyamide 6, poly-

amide 11, and polyamide 12 are particularly preferred. A preferable polyamide resin in light of versatility is nylon 6.

Specific examples of polyamide resins include trade names "Novamid ST220", "Novamid 1010C2", and "Novamid ST145", manufactured by Mitsubishi Engineering-Plastics Corporation; trade name "Pebax 4033SA" manufactured by Arkema Inc.; trade names "UBE Nylon 10181", "UBE Nylon 1030J", "UBESTA P3014U", "UBESTA 3035JU6", and "UBESTA PAE1200U2", manufactured by Ube Industries, Ltd.; trade names "Zytel 5N716" and "Zytel ST811HS" manufactured by E. I. du Pont de Nemours and Company; trade names "Amilan U441", "Amilan U328", and "Amilan U141", manufactured by Toray Industries Inc.; and trade name "Leona 1300S" manufactured by Asahi Kasei Corporation.

When an ionomer resin and a polyamide resin are used in combination, the ionomer resin is included as the principal component of the base polymer. The proportion of the ionomer resin to the entire base polymer is preferably equal to or greater than 50% by weight, more preferably equal to or greater than 65% by weight, and particularly preferably equal to or greater than 70% by weight. The base resin including an ionomer resin and a polyamide resin may further include another resin.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the mid layer 6 in an adequate amount. Powder of a metal with a high specific gravity may be included as a filler. Specific examples of metals with a high specific gravity include tungsten and molybdenum. The amount of the filler is determined as appropriate so that the intended specific gravity of the mid layer 6 is accomplished.

The thickness  $T_m$  of the mid layer 6 can be appropriately adjusted such that a condition described later for the volume  $V_m$  of the mid layer 6 is met. In light of durability, the thickness  $T_m$  is preferably equal to or greater than 0.8 mm and more preferably equal to or greater than 0.9 mm. In light of resilience performance, the thickness  $T_m$  is preferably equal to or less than 1.4 mm and more preferably equal to or less than 1.2 mm. Preferably, a sphere consisting of the core 4 and the mid layer 6 has a diameter of 39.1 mm or greater but 41.5 mm or less.

The volume  $V_m$  of the mid layer 6 can be appropriately adjusted such that the condition described later is met. Preferably, the volume  $V_m$  is equal to or greater than 4800  $\text{mm}^3$  but equal to or less than 5200  $\text{mm}^3$ .

In light of suppression of spin upon a shot with a driver, the mid layer 6 has a Shore D hardness  $H_m$  of preferably 68 or greater, more preferably 69 or greater, and particularly preferably 70 or greater. In light of feel at impact, the hardness  $H_m$  is preferably equal to or less than 80 and more preferably equal to or less than 76.

In the present invention, the hardness of the mid layer 6 is measured according to the standards of "ASTM-D 2240-68". For the measurement, an automated rubber hardness measurement machine (trade name "P1", manufactured by Kobunshi Keiki Co., Ltd.), to which a Shore D type hardness scale is mounted, is used. For the measurement, a sheet that is formed by hot press, is formed from the same material as that of the mid layer 6, and has a thickness of about 2 mm is used. Prior to the measurement, a sheet is kept at 23°C. for two weeks. At the measurement, three sheets are stacked.

In light of feel at impact, the sphere consisting of the core 4 and the mid layer 6 has an amount of compressive

deformation of preferably 2.0 mm or greater, more preferably 2.2 mm or greater, and particularly preferably 2.4 mm or greater. In light of resilience performance, the amount of compressive deformation of the sphere is preferably equal to or less than 4.0 mm, more preferably equal to or less than 3.6 mm, and particularly preferably equal to or less than 3.4 mm.

For the inner cover 8, a resin composition is suitably used. Examples of the base resin of the resin composition include 10 ionomer resins, polystyrenes, polyesters, polyamides, and polyolefins.

Particularly preferable base polymers are ionomer resins. The ionomer resin described above for the mid layer 6 can be used. The golf ball 2 including the inner cover 8 that 15 includes an ionomer resin has excellent resilience performance.

An ionomer resin and another resin may be used in combination for the inner cover 8. In this case, the principal component of the base polymer is preferably the ionomer 20 resin. Specifically, the proportion of the ionomer resin to the entire base polymer is preferably equal to or greater than 60% by weight and more preferably equal to or greater than 70% by weight.

An example of the other resin used in combination with 25 the ionomer resin is a styrene block-containing thermoplastic elastomer. The styrene block-containing thermoplastic elastomer includes a polystyrene block as a hard segment, and a soft segment. A typical soft segment is a diene block. Examples of styrene block-containing thermoplastic elastomers include styrene-butadiene-styrene block copolymers (SBS), styrene-isoprene-styrene block copolymers (SIS), styrene-isoprene-butadiene-styrene block copolymers (SIBS), hydrogenated SBS, hydrogenated SIS, and hydrogenated SIBS. Examples of hydrogenated SBS include 30 styrene-ethylene-butylene-styrene block copolymers (SEBS). Examples of hydrogenated SIS include styrene-ethylene-propylene-styrene block copolymers (SEPS). Examples of hydrogenated SIBS include styrene-ethylene-ethylene-propylene-styrene block copolymers (SEEPS).

40 In light of resilience performance of the golf ball 2, the content of the styrene component in the thermoplastic elastomer is preferably equal to or greater than 10% by weight, more preferably equal to or greater than 12% by weight, and particularly preferably equal to or greater than 15% by weight. In light of feel at impact of the golf ball 2, the content is preferably equal to or less than 50% by weight, more preferably equal to or less than 47% by weight, and particularly preferably equal to or less than 45% by weight.

In the present invention, styrene block-containing thermoplastic elastomers include an alloy of an olefin and one or 50 more members selected from the group consisting of SBS, SIS, SIBS, and hydrogenated products thereof. The olefin component in the alloy is presumed to contribute to improvement of compatibility with another base polymer.

55 Use of this alloy improves the resilience performance of the golf ball 2. An olefin having 2 to 10 carbon atoms is preferably used. Examples of suitable olefins include ethylene, propylene, butene, and pentene. Ethylene and propylene are particularly preferred.

60 Specific examples of polymer alloys include trade names "Rabalon T3221C", "Rabalon T3339C", "Rabalon SJ4400N", "Rabalon SJ5400N", "Rabalon SJ6400N", "Rabalon SJ7400N", "Rabalon SJ8400N", "Rabalon SJ9400N", and "Rabalon SR04", manufactured by Mitsubishi Chemical Corporation. Other specific examples of styrene block-containing thermoplastic elastomers include trade name "Epofriend A1010" manufactured by Daicel

## 11

Chemical Industries, Ltd., and trade name "Septon HG-252" manufactured by Kuraray Co., Ltd.

The inner cover **8** may include a highly elastic resin. The highly elastic resin described above for the mid layer **6** can be used.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the resin composition of the inner cover **8** in an adequate amount.

In light of a spin suppression effect upon a shot with a driver, the inner cover **8** has a Shore D hardness Hinc of preferably 40 or greater and more preferably 48 or greater. The flight distance of the golf ball **2** is large. In light of approach performance of the golf ball **2**, the hardness Hinc is preferably equal to or less than 60 and more preferably equal to or less than 56. When the golf ball **2** is hit with a short iron, the spin rate is high. The hardness Hinc is measured by the same method as that for the hardness Hm.

The thickness Tinc of the inner cover **8** can be appropriately adjusted such that a condition described later for the volume Vinc of the inner cover **8** is met. Preferably, the thickness Tinc is equal to or greater than 0.5 mm but equal to or less than 1.2 mm. In the golf ball **2** including the inner cover **8** having a thickness Tinc of 0.5 mm or greater, the shock by a hit is alleviated, and thus the durability is improved. In this respect, the thickness Tinc is more preferably equal to or greater than 0.7 mm. The golf ball **2** including the inner cover **8** having a thickness Tinc of 1.2 mm or less includes a relatively large core **4**. The golf ball **2** exerts sufficient resilience performance. In this respect, the thickness Tinc is more preferably equal to or less than 1.0 mm. Preferably, a sphere consisting of the core **4**, the mid layer **6**, and the inner cover **8** has a diameter of 42.1 mm or greater but 42.6 mm or less.

The volume Vinc of the inner cover **8** can be appropriately adjusted such that the condition described later is met. Preferably, the volume Vinc is equal to or greater than 3500 mm<sup>3</sup> but equal to or less than 4500 mm<sup>3</sup>.

In light of feel at impact, the sphere consisting of the core **4**, the mid layer **6**, and the inner cover **8** has an amount of compressive deformation of preferably 2.0 mm or greater, more preferably 2.2 mm or greater, and particularly preferably 2.4 mm or greater. In light of resilience performance, the amount of compressive deformation of the sphere is preferably equal to or less than 4.0 mm, more preferably equal to or less than 3.6 mm, and particularly preferably equal to or less than 3.4 mm.

For forming the inner cover **8**, known methods such as injection molding, compression molding, and the like can be used.

For the outer cover **12**, a resin composition is suitably used. A preferable base resin of the resin composition is a urethane resin or a urea resin. The principal component of the urethane resin is a polyurethane. The polyurethane is flexible. When the golf ball **2** that includes the outer cover **12** formed from the resin composition that includes the polyurethane is hit with a short iron, the spin rate is high. The outer cover **12** formed from this resin composition contributes to approach performance upon a shot with a short iron. The polyurethane also contributes to scuff resistance of the outer cover **12**. Furthermore, the polyurethane can contribute to excellent feel at impact when the golf ball **2** is hit with a putter or a short iron.

In light of ease of forming the outer cover **12**, a preferable base resin is a thermoplastic polyurethane elastomer. The

## 12

thermoplastic polyurethane elastomer includes a polyurethane component as a hard segment, and a polyester component or a polyether component as a soft segment. Examples of isocyanates for the polyurethane component include alicyclic diisocyanates, aromatic diisocyanates, and aliphatic diisocyanates. Two or more diisocyanates may be used in combination.

Examples of alicyclic diisocyanates include 4,4'-dicyclohexylmethane diisocyanate (H<sub>12</sub>MDI), 1,3-bis(isocyanatomethyl)cyclohexane (H<sub>6</sub>XDI), isophorone diisocyanate (IPDI), and trans-1,4-cyclohexane diisocyanate (CHDI). In light of versatility and processability, H<sub>12</sub>MDI is preferred.

Examples of aromatic diisocyanates include 4,4'-diphenylmethane diisocyanate (MDI) and toluene diisocyanate (TDI). Examples of aliphatic diisocyanates include hexamethylene diisocyanate (HDI).

Alicyclic diisocyanates are particularly preferred. Since an alicyclic diisocyanate does not have any double bond in the main chain, the alicyclic diisocyanate suppresses yellowing of the outer cover **12**. In addition, since an alicyclic diisocyanate has excellent strength, the alicyclic diisocyanate suppresses damage of the outer cover **12**.

Specific examples of thermoplastic polyurethane elastomers include trade names "Elastollan NY80A", "Elastollan NY82A", "Elastollan NY84A", "Elastollan NY85A", "Elastollan NY88A", "Elastollan NY90A", "Elastollan NY97A", "Elastollan NY585", "Elastollan XKP016N", "Elastollan 1195ATR", "ElastollanET890A", and "Elastollan ET88050", manufactured by BASF Japan Ltd.; and trade names "RESAMINE P458LS" and "RESAMINE PS62490", manufactured by Dainichiseika Color & Chemicals Mfg. Co., Ltd. From the standpoint that a low hardness of the outer cover **12** can be achieved, "Elastollan NY80A", "Elastollan NY82A", "Elastollan NY84A", "Elastollan NY85A", "Elastollan NY90A", and "Elastollan NY97A" are particularly preferred.

A thermoplastic polyurethane elastomer and another resin may be used in combination. Examples of the resin that can be used in combination include thermoplastic polyester elastomers, thermoplastic polyamide elastomers, thermoplastic polyolefin elastomers, styrene block-containing thermoplastic elastomers, and ionomer resins. When a thermoplastic polyurethane elastomer and another resin are used in combination, the thermoplastic polyurethane elastomer is included as the principal component of the base polymer, in light of spin performance and scuff resistance. The proportion of the thermoplastic polyurethane elastomer to the entire base polymer is preferably equal to or greater than 50% by weight, more preferably equal to or greater than 70% by weight, and particularly preferably equal to or greater than 85% by weight.

According to need, a coloring agent such as titanium dioxide, a filler such as barium sulfate, a dispersant, an antioxidant, an ultraviolet absorber, a light stabilizer, a fluorescent material, a fluorescent brightener, and the like are included in the outer cover **12** in an adequate amount.

The outer cover **12** preferably has a Shore D hardness Houg of 36 or less. The golf ball **2** including the outer cover **12** having a hardness Houg of 36 or less has excellent approach performance. In this respect, the hardness Houg is more preferably equal to or less than 32 and particularly preferably equal to or less than 30. In light of flight distance upon a shot with a driver, the hardness Houg is preferably equal to or greater than 10 and more preferably equal to or greater than 15. The hardness Houg is measured by the same measurement method as that for the hardness Hm and the hardness Hinc.

## 13

When the golf ball **2** is hit, the outer cover **12** including the polyurethane absorbs the shock. This absorption achieves soft feel at impact. Particularly, when the golf ball **2** is hit with a short iron or a putter, the flexible outer cover **12** achieves excellent feel at impact.

The thickness Touc of the outer cover **12** can be appropriately adjusted such that a condition described later for the volume Vouc of the outer cover **12** is met. In light of high flight distance performance upon a shot with a driver, the thickness Touc is preferably equal to or less than 0.6 mm. The thickness Touc is more preferably equal to or less than 0.4 mm and particularly preferably equal to or less than 0.3 mm. In light of durability and approach performance, the thickness Touc is preferably equal to or greater than 0.1 mm.

The volume Vouc of the outer cover **12** can be appropriately adjusted such that the condition described later is met. Preferably, the volume Vouc is equal to or greater than 1500 mm<sup>3</sup> but equal to or less than 3200 mm<sup>3</sup>.

In light of feel at impact, the golf ball **2** has an amount of compressive deformation of preferably 2.0 mm or greater and more preferably 2.2 mm or greater. In light of resilience performance, the amount of compressive deformation of the golf ball **2** is preferably equal to or less than 3.6 mm and more preferably equal to or less than 3.2 mm.

For forming the outer cover **12**, known methods such as injection molding, compression molding, and the like can be used. When forming the outer cover **12**, the dimples **14** are formed by pimples formed on the cavity face of a mold.

In light of durability, the golf ball **2** that further includes the reinforcing layer **10** between the inner cover **8** and the outer cover **12** is preferred. The reinforcing layer **10** is positioned between the inner cover **8** and the outer cover **12**. The reinforcing layer **10** firmly adheres to the inner cover **8** and also to the outer cover **12**. The reinforcing layer **10** suppresses separation of the outer cover **12** from the inner cover **8**. The golf ball **2** includes a relatively thin outer cover **12**. When the thin cover is hit with the edge of a clubface, a wrinkle is likely to occur. The reinforcing layer **10** suppresses occurrence of a wrinkle to improve the durability of the golf ball **2**.

As the base polymer of the reinforcing layer **10**, a two-component curing type thermosetting resin is suitably used. Specific examples of two-component curing type thermosetting resins include epoxy resins, urethane resins, acrylic resins, polyester resins, and cellulose resins. In light of strength and durability of the reinforcing layer **10**, two-component curing type epoxy resins and two-component curing type urethane resins are preferred.

A two-component curing type epoxy resin is obtained by curing an epoxy resin with a polyamide type curing agent. Examples of epoxy resins used in two-component curing type epoxy resins include bisphenol A type epoxy resins, bisphenol F type epoxy resins, and bisphenol AD type epoxy resins. In light of balance among flexibility, chemical resistance, heat resistance, and toughness, bisphenol A type epoxy resins are preferred. Specific examples of the polyamide type curing agent include polyamide amine curing agents and modified products thereof. In a mixture of an epoxy resin and a polyamide type curing agent, the ratio of the epoxy equivalent of the epoxy resin to the amine active hydrogen equivalent of the polyamide type curing agent is preferably equal to or greater than 1.0/1.4 but equal to or less than 1.0/1.0.

A two-component curing type urethane resin is obtained by a reaction of a base material and a curing agent. A two-component curing type urethane resin obtained by a reaction of a base material containing a polyol component

## 14

and a curing agent containing a polyisocyanate or a derivative thereof, and a two-component curing type urethane resin obtained by a reaction of a base material containing an isocyanate group-terminated urethane prepolymer and a curing agent having active hydrogen, can be used. Particularly, a two-component curing type urethane resin obtained by a reaction of a base material containing a polyol component and a curing agent containing a polyisocyanate or a derivative thereof, is preferred.

The reinforcing layer **10** may include additives such as a coloring agent (typically, titanium dioxide), a phosphate-based stabilizer, an antioxidant, a light stabilizer, a fluorescent brightener, an ultraviolet absorber, an anti-blocking agent, and the like. The additives may be added to the base material of the two-component curing type thermosetting resin, or may be added to the curing agent of the two-component curing type thermosetting resin.

The reinforcing layer **10** is obtained by applying, to the surface of the inner cover **8**, a liquid that is prepared by dissolving or dispersing the base material and the curing agent in a solvent. In light of workability, application with a spray gun is preferred. After the application, the solvent is volatilized to permit a reaction of the base material with the curing agent, thereby forming the reinforcing layer **10**. Examples of preferable solvents include toluene, isopropyl alcohol, xylene, methyl ethyl ketone, methyl isobutyl ketone, ethylene glycol monomethyl ether, ethylbenzene, propylene glycol monomethyl ether, isobutyl alcohol, and ethyl acetate.

In light of suppression of a wrinkle, the reinforcing layer **10** has a thickness of preferably 3 µm or greater and more preferably 5 µm or greater. In light of ease of forming the reinforcing layer **10**, the thickness is preferably equal to or less than 100 µm, more preferably equal to or less than 50 µm, and further preferably equal to or less than 20 µm. The thickness is measured by observing a cross section of the golf ball **2** with a microscope. When the inner cover **8** has concavities and convexities on its surface from surface roughening, the thickness is measured at a convex part.

In light of suppression of a wrinkle, the reinforcing layer **10** has a pencil hardness of preferably 4B or greater and more preferably B or greater. In light of reduced loss of the power transmission from the outer cover **12** to the inner cover **8** upon hitting the golf ball **2**, the pencil hardness of the reinforcing layer **10** is preferably equal to or less than 3H. The pencil hardness is measured according to the standards of "JIS K5400".

When the inner cover **8** and the outer cover **12** sufficiently adhere to each other so that a wrinkle is unlikely to occur, the reinforcing layer **10** may not be provided.

In light of feel at impact, the golf ball **2** has an amount of compressive deformation of preferably 2.0 mm or greater and more preferably 2.2 mm or greater. In light of resilience performance, the amount of compressive deformation of the golf ball **2** is preferably equal to or less than 3.6 mm and more preferably equal to or less than 3.2 mm.

In measurement of the amount of compressive deformation, a sphere (the golf ball **2**, the core **4**, or the like) is placed on a hard plate made of metal. Next, a cylinder made of metal gradually descends toward the sphere. The sphere, squeezed between the bottom face of the cylinder and the hard plate, becomes deformed. A migration distance of the cylinder, starting from the state in which an initial load of 98 N is applied to the sphere up to the state in which a final load of 1274 N is applied thereto, is measured.

In the golf ball **2** according to the present invention, the hardness is lower in order of the mid layer **6**, the inner cover

## 15

8, and the outer cover 12. In other words, in the golf ball 2, the hardness does not rapidly change from the outside of the core 4 toward the ball surface. When the golf ball 2 is hit, no local load is applied thereto. The golf ball 2 has excellent durability.

In the golf ball 2, the hardness Hinc of the inner cover 8 is less than the hardness Hm of the mid layer 6. The golf ball 2 has excellent feel at impact and durability.

From the standpoint that favorable feel at impact is obtained, the difference (Hm-Hinc: between the hardness Hm of the mid layer 6 and the hardness Hinc of the inner cover 8) is preferably equal to or greater than 8 and particularly preferably equal to or greater than 14. In light of durability, the difference (Hm-Hinc) is preferably equal to or less than 30.

The hardness Houc of the outer cover 12 of the golf ball 2 is less than the hardness Hinc of the inner cover 8. When the golf ball 2 is hit with a driver, the sphere consisting of the core 4, the mid layer 6, and the inner cover 8 becomes significantly distorted since the head speed is high. In the core 4, the outer-hard/inner-soft structure is formed. The core 4 suppresses a spin rate. The golf ball 2 is launched at a high speed due to deformation and restoration of the core 4. The suppression of the spin rate and the high launch speed achieve a large flight distance. When the golf ball 2 is hit with a short iron, the sphere consisting of the core 4, the mid layer 6, and the inner cover 8 becomes less distorted since the head speed is low. When the golf ball 2 is hit with a short iron, the behavior of the golf ball 2 mainly depends on the outer cover 12. In the golf ball 2, since the outer cover 12 is flexible, a slip between the golf ball 2 and a clubface is suppressed. Due to the suppression of the slip, a high spin rate is obtained. The high spin rate achieves excellent approach performance.

In light of approach performance, the difference (Hinc-Houc) between the hardness Hinc of the inner cover 8 and the hardness Houc of the outer cover 12 is preferably equal to or greater than 15 and more preferably equal to or greater than 20. In the golf ball 2 that meets this condition, a spin rate is high upon an approach shot. In light of durability, the difference (Hinc-Houc) is preferably equal to or less than 45 and more preferably equal to or less than 40.

The difference (Hm-Houc) between the hardness Hm of the mid layer 6 and the hardness Houc of the outer cover 12 is greater than 25. In the golf ball 2 that meets this condition, a spin rate can be sufficiently suppressed upon a shot with a driver. When the golf ball 2 is hit with a driver, the flight distance is large. In this respect, the difference (Hm-Houc) is more preferably equal to or greater than 27 and particularly preferably equal to or greater than 29. In light of durability, the difference (Hm-Houc) is preferably equal to or less than 55 and more preferably equal to or less than 50.

In the golf ball 2 according to the present invention, the mid layer 6, the inner cover 8, and the outer cover 12 are arranged in appropriate balance from the outside of the core 4 to the ball surface. In the golf ball 2 which is a sphere, variation of the volume of each layer greatly influences various performance characteristics. In the golf ball 2 according to the present invention, the mid layer 6, the inner cover 8, and the outer cover 12 are arranged on the basis of the volume of each layer. In the golf ball 2, both high flight distance performance and approach performance can be achieved on a high level without impairing feel at impact and durability.

The volume Vm of the mid layer 6 of the golf ball 2 is greater than the volume Vinc of the inner cover 8. The volume Vinc of the inner cover 8 is greater than the volume

## 16

Vouc of the outer cover 12. In other words, in the golf ball 2, the volume is lower in order of the mid layer 6, the inner cover 8, and the outer cover 12. As described above, in the golf ball 2, the hardness is lower in order of the mid layer 6, the inner cover 8, and the outer cover 12. In the golf ball 2, the volume of the most flexible outer cover 12 is the lowest. In the golf ball 2, excessive spin due to the flexible outer cover 12 is suppressed.

Preferably, the ratio  $[(Vm+Vinc+Vouc)/V]$  of the sum <sup>10</sup> (Vm+Vinc+Vouc) of the volume Vm, the volume Vinc, and the volume Vouc relative to the volume V of the entirety of the golf ball 2 is less than 0.30. In the golf ball 2, the sufficiently large core 4 is formed, and thus excellent resilience performance of the core 4 can be exerted. In this <sup>15</sup> respect, the ratio  $[(Vm+Vinc+Vouc)/V]$  is more preferably equal to or less than 0.29 and particularly preferably equal to or less than 0.28.

Preferably, the ratio  $(Vm/Vouc)$  of the volume Vm relative to the volume Vouc is greater than 1.50. In the golf ball <sup>20</sup> 2 having a ratio  $(Vm/Vouc)$  of greater than 1.50, the most flexible outer cover 12 and the mid layer 6 harder than the outer cover 12 are arranged in a well-balanced manner. In the golf ball 2, although the outer cover 12 is flexible, a spin rate can be sufficiently suppressed upon a shot with a driver. <sup>25</sup> In this respect, the ratio  $(Vm/Vouc)$  is more preferably equal to or greater than 1.70 and particularly preferably equal to or greater than 2.50.

Preferably, the product  $(Vm*Hm)$  of the hardness Hm and the volume Vm of the mid layer 6 and the product <sup>30</sup>  $(Vouc*Houc)$  of the hardness Houc and the volume Vouc of the outer cover 12 meet the following relationship.

$$[(Vm*Hm)/(Vouc*Houc)] > 3.0$$

In the golf ball 2 that meets the above relationship, the <sup>35</sup> balance between the mid layer 6 and the outer cover 12 is appropriate. In the golf ball 2, although the outer cover 12 is flexible, a spin rate can be sufficiently suppressed upon a shot with a driver. In this respect,  $[(Vm*Hm)/(Vouc*Houc)]$  is more preferably equal to or greater than 4.0 and particularly preferably equal to or greater than 6.0.

More preferably, the ratio  $(Vouc/V)$  of the volume Vouc relative to the volume V is less than 0.08. In the golf ball 2, suppression of spin upon a shot with a driver is not impaired due to the presence of the flexible outer cover 12. In this <sup>45</sup> respect, the ratio  $(Vouc/V)$  is particularly preferably equal to or less than 0.04. In light of durability, the ratio  $(Vouc/V)$  is particularly preferably equal to or greater than 0.01.

## EXAMPLES

The following will show the effects of the present invention by means of Examples, but the present invention should not be construed in a limited manner based on the description of these Examples.

## Example 1

A rubber composition was obtained by kneading 100 parts by weight of a high-cis polybutadiene (trade name "BR-730", manufactured by JSR Corporation), 32 parts by weight of zinc diacrylate (trade name "Sanceler SR", manufactured by SANSHIN CHEMICAL INDUSTRY CO., LTD.), 5 parts by weight of zinc oxide, an appropriate amount of barium sulfate, 0.20 parts by weight of 2-thionaphthol (manufactured by Tokyc Chemical Industry Co., Ltd.), 0.90 parts by weight of dicumyl peroxide (trade name "Percumyl D" manufactured by NOF Corporation), and 2.0 parts by weight

of zinc octoate (a product of Mitsuwa Chemicals Co., Ltd.). This rubber composition was placed into a mold including upper and lower mold halves each having a hemispherical cavity, and heated at 150° C. for 20 minutes to obtain a spherical core with a diameter of 38.5 mm.

A resin composition was obtained by kneading 50 parts by weight of an ionomer resin (The aforementioned "Surlyn 8150"), 50 parts by weight of another ionomer resin (the aforementioned "Himilan 9150"), and 3 parts by weight of titanium dioxide with a twin-screw kneading extruder. The extruding conditions were a screw diameter of 45 mm, a screw rotational speed of 200 rpm, a screw L/D of 35, and a die temperature of 160 to 230° C. The core was placed into a mold. The resin composition was injected around the core by injection molding to form a mid layer with a thickness of 1.0 mm.

A resin composition was obtained by kneading 31.5 parts by weight of an ionomer resin (the aforementioned "Himilan AM7337"), 38.5 parts by weight of another ionomer resin (the aforementioned "Himilan AM7329"), 16 parts by weight of an ethylene-methacrylic acid copolymer (trade name "NUCREL N1050H", manufactured by Du Pont-MITSUI POLYCHEMICALS Co., Ltd.), 14 parts by weight of a styrene block-containing thermoplastic elastomer (the aforementioned "Rabalon T3221C"), and 3 parts by weight of titanium dioxide with a twin-screw kneading extruder under the above extruding conditions. The sphere consisting of the core and the mid layer was placed into a mold. The resin composition was injected around the sphere by injection molding to form an inner cover with a thickness of 0.8 mm.

A paint composition (trade name "POLIN 750LE", manufactured by SHINTO PAINT CO., LTD.) including a two-component curing type epoxy resin as a base polymer was prepared. The base material liquid of this paint composition includes 30 parts by weight of a bisphenol A type solid epoxy resin and 70 parts by weight of a solvent. The curing agent liquid of this paint composition includes 40 parts by weight of a modified polyamide amine, 55 parts by weight of a solvent, and 5 parts by weight of titanium dioxide. The weight ratio of the base material liquid to the curing agent liquid is 1/1. This paint composition was applied to the surface of the inner cover with an air gun, and kept at 23° C. for 12 hours to obtain a reinforcing layer with a thickness of 10 µm.

A resin composition was obtained by kneading 100 parts by weight of a thermoplastic polyurethane elastomer (the aforementioned "Elastollan NY82A"), 0.2 parts by weight of a hindered amine light stabilizer (trade name "TINUVIN 770", manufactured by Ciba Japan K.K.), 4 parts by weight of titanium dioxide, and 0.04 parts by weight of ultramarine blue with a twin-screw kneading extruder under the above extruding conditions. Half shells were formed from this resin composition by compression molding. The sphere consisting of the core, the mid layer, the inner cover, and the reinforcing layer was covered with two of these half shells. The sphere and the half shells were placed into a final mold that includes upper and lower mold halves each having a hemispherical cavity and that has a large number of pimples on its cavity face. An outer cover was obtained by compression molding. The thickness of the cover was 0.3 mm. Dimples having a shape that is the inverted shape of the pimples were formed on the cover. The surface of the cover was polished. A clear paint including a two-component curing type polyurethane as a base material was applied to

this cover with an air gun, and was dried and cured to obtain a golf ball of Example 1 with a diameter of 42.7 mm and a weight of 45.6 g.

5 Examples 2 to 8 and Comparative Examples 1 to 10

Golf balls of Examples 2 to 8 and Comparative Examples 1 to 10 were obtained in the same manner as Example 1, 10 except the specifications of the core, the mid layer, the inner cover, and the outer cover were as shown in Tables 4 to 6 below. The rubber composition of the core is shown in detail in Table 1 below. The resin compositions of the mid layer and the inner cover are shown in detail in Table 2 below. The 15 resin composition of the outer cover is shown in detail in Table 3 below. The cover of each of the golf balls according to Comparative Examples 5 and 6 is composed of a single layer.

[Resilience Coefficient]

20 A metallic cylinder having a weight of 198.4 g was caused to collide against a golf ball at a speed of 45 m/sec. The speeds of the metallic cylinder and the golf ball before and after the collision were measured, and a resilience coefficient was calculated based on the speeds. An average value 25 obtained for 12 golf balls is shown as an index in Tables 7 to 9 below. The higher the index is, the more excellent the resilience performance of the golf ball is.

[Shot with Driver (W#1)]

20 A driver with a titanium head (trade name "XXIO", 30 manufactured by DUNLOP SPORTS CO. LTD., shaft hardness: S, loft angle: 10.0°) was attached to a swing machine manufactured by Golf Laboratories, Inc. A golf ball was hit under the condition of a head speed of 45 m/sec. The ball speed and the spin rate immediately after the hit and the 35 flight distance from the launch point to the stop point were measured. The average value of data obtained by 10 measurements is shown in Tables 7 to 9 below.

[Hit with Sand Wedge (SW)]

40 A sand wedge (trade name "XXIO", manufactured by 40 DUNLOP SPORTS CO. LTD., shaft hardness: R, loft angle: 56.0°) was attached to a swing machine manufactured by True Temper Co. A golf ball was hit under the condition of a head speed of 21 m/sec. The backspin rate was measured immediately after the hit. The average value of data obtained by 10 measurements is shown in Tables 7 to 9 below.

[Durability]

40 A driver with a titanium head (trade name "XXIO", 50 manufactured by DUNLOP SPORTS CO. LTD., shaft hardness: S, loft angle: 10.0°) was attached to a swing robot M/C manufactured by True Temper Co. A golf ball having been 50 kept at 23° C. for 12 hours was used for the measurement. The golf ball was repeatedly hit under the condition of a head speed of 45 m/sec. The number of hits required to break the golf ball was measured. An average value obtained for 55 12 golf balls is shown as an index in Tables 7 to 9 below. The higher the index is, the more excellent the durability of the golf ball is.

[Feel at Impact]

60 A golf player hit golf balls with a driver (trade name "XXIO", manufactured by DUNLOP SPORTS CO. LTD., shaft hardness: S, loft angle: 10.0°) and categorized the evaluation on the basis of the following criteria. The results are shown in Tables 7 to 9 below.

A: very favorable (soft)

B: favorable (slightly soft)

C: slightly poor (slightly hard)

D: poor (hard)

TABLE 1

| Type             | Composition of Core |      |      |      |      |
|------------------|---------------------|------|------|------|------|
|                  | 1                   | 2    | 3    | 4    | 5    |
| BR-730           | 100                 | 100  | 100  | 100  | 100  |
| Sanceler SR      | 32                  | 31   | 33   | 34   | 30   |
| Zinc oxide       | 5                   | 5    | 5    | 5    | 5    |
| Barium sulfate   | *                   | *    | *    | *    | *    |
| 2-thionaphthol   | 0.20                | 0.20 | 0.20 | 0.20 | 0.20 |
| Dicumyl peroxide | 0.90                | 0.90 | 0.90 | 0.90 | 0.90 |
| Zinc octoate     | 2.0                 | 2.0  | 2.0  | 2.0  | 0    |

\* Appropriate amount

The details of the compounds listed in Table 1 are as follows.

BR-730: a high-cis polybutadiene manufactured by JSR Corporation (cis-1,4-bond content: 96% by weight, 1,2-vinyl bond content: 1.3% by weight, Mooney viscosity (ML1+4 (100° C.)):55, molecular weight distribution (Mw/Mn):3)

Sanceler SR: zinc diacrylate manufactured by SANSHIN CHEMICAL INDUSTRY CO., LTD. (a product coated with 10% by weight of stearic acid)

Zinc oxide: trade name "Ginrei R" manufactured by Toho Zinc Co., Ltd.

Barium sulfate: trade name "Barium Sulfate BD" manufactured by Sakai Chemical Industry Co., Ltd.

2-thionaphthol: a product of Tokyo Chemical Industry Co., Ltd.

Dicumyl peroxide: trade name "Percumyl D" manufactured by NOF Corporation

Zinc octoate: a product of Mitsuwa Chemicals Co., Ltd.

TABLE 2

| Type              | Compositions and Hardnesses of Mid Layer and Inner Cover |      |    |      |    |    |
|-------------------|----------------------------------------------------------|------|----|------|----|----|
|                   | a                                                        | b    | c  | d    | e  | f  |
| Surlyn 8150       | 50                                                       | 32.5 | —  | —    | —  | —  |
| Surlyn 9150       | 50                                                       | 32.5 | —  | —    | —  | —  |
| Nylon 6           | —                                                        | 35   | —  | —    | —  | —  |
| Himilan AM7337    | —                                                        | —    | 55 | 31.5 | 24 | 44 |
| Himilan AM7329    | —                                                        | —    | 45 | 38.5 | 30 | 50 |
| NUCREL NI1050H    | —                                                        | —    | —  | 16   | 16 | —  |
| Rabalon T3221C    | —                                                        | —    | —  | 14   | 30 | 6  |
| Titanium dioxide  | 3                                                        | 3    | 3  | 3    | 3  | 3  |
| Hardness(Shore D) | 70                                                       | 72   | 65 | 55   | 43 | 62 |

The details of the compounds listed in Table 2 are as follows.

Nylon 6: a polyamide resin manufactured by Toray Industries Inc.

Titanium dioxide: a product of Ishihara Sangyo Kaisha, Ltd.

TABLE 3

| Type              | Composition and Hardness of Outer Cover |      |      |      |
|-------------------|-----------------------------------------|------|------|------|
|                   | A                                       | B    | C    | D    |
| Elastollan NY82A  | 100                                     | —    | —    | 10   |
| Elastollan NY85A  | —                                       | 50   | —    | —    |
| Elastollan NY90A  | —                                       | 50   | —    | —    |
| Elastollan NY97A  | —                                       | —    | 100  | 90   |
| TINUVIN 770       | 0.2                                     | 0.2  | 0.2  | 0.2  |
| Titanium dioxide  | 4                                       | 4    | 4    | 4    |
| Ultramarine blue  | 0.04                                    | 0.04 | 0.04 | 0.04 |
| Hardness(Shore D) | 29                                      | 36   | 47   | 45   |

TABLE 4

| 5                          | Configuration of Golf Ball |       |       |       |       |       |
|----------------------------|----------------------------|-------|-------|-------|-------|-------|
|                            | Ex. 1                      | Ex. 2 | Ex. 3 | Ex. 4 | Ex. 5 | Ex. 6 |
| <u>Core</u>                |                            |       |       |       |       |       |
| Composition                | 1                          | 1     | 1     | 2     | 5     | 3     |
| Vul. temp. (° C.)          | 150                        | 150   | 150   | 150   | 150   | 150   |
| 10 Vul. time (min)         | 20                         | 20    | 20    | 20    | 20    | 20    |
| Diameter I (mm)            | 38.5                       | 38.1  | 38.5  | 38.5  | 38.5  | 38.5  |
| Ho (JIS-C)                 | 59                         | 59    | 59    | 58    | 64    | 60    |
| Hs (JIS-C)                 | 86                         | 86    | 86    | 85    | 83    | 87    |
| (Hs - Ho)                  | 27                         | 27    | 27    | 27    | 19    | 27    |
| 15 <u>Mid layer</u>        |                            |       |       |       |       |       |
| Composition                | a                          | a     | a     | b     | a     | c     |
| Hm (Shore D)               | 70                         | 70    | 70    | 72    | 70    | 65    |
| Thickness (mm)             | 1.00                       | 1.00  | 1.00  | 1.00  | 1.00  | 1.00  |
| Diameter II (mm)           | 40.5                       | 40.1  | 40.5  | 40.5  | 40.5  | 40.5  |
| 20 Vm (mm <sup>3</sup> )   | 4900                       | 4802  | 4900  | 4900  | 4900  | 4900  |
| <u>Inner cover</u>         |                            |       |       |       |       |       |
| Composition                | d                          | d     | d     | d     | d     | d     |
| Hinc (Shore D)             | 55                         | 55    | 55    | 55    | 55    | 55    |
| Thickness (mm)             | 0.80                       | 0.80  | 0.80  | 0.80  | 0.80  | 0.80  |
| Diameter III (mm)          | 42.1                       | 41.7  | 42.1  | 42.1  | 42.1  | 42.1  |
| 25 Vinc (mm <sup>3</sup> ) | 4285                       | 4203  | 4285  | 4285  | 4285  | 4285  |
| <u>Outer cover</u>         |                            |       |       |       |       |       |
| Composition                | A                          | A     | B     | A     | A     | A     |
| 30 Houc (Shore D)          | 29                         | 29    | 36    | 29    | 29    | 29    |
| Thickness (mm)             | 0.30                       | 0.50  | 0.30  | 0.30  | 0.30  | 0.30  |
| Diameter IV (mm)           | 42.7                       | 42.7  | 42.7  | 42.7  | 42.7  | 42.7  |
| 35 Vouc (mm <sup>3</sup> ) | 1694                       | 2796  | 1694  | 1694  | 1694  | 1694  |

35

TABLE 5

| 35                         | Configuration of Golf Ball |       |            |            |            |            |
|----------------------------|----------------------------|-------|------------|------------|------------|------------|
|                            | Ex. 7                      | Ex. 8 | Com. Ex. 1 | Com. Ex. 2 | Com. Ex. 3 | Com. Ex. 4 |
| <u>Core</u>                |                            |       |            |            |            |            |
| Composition                | 1                          | 1     | 1          | 2          | 1          | 2          |
| Vul. temp. (° C.)          | 150                        | 150   | 150        | 150        | 150        | 150        |
| 40 Vul. time (min)         | 20                         | 20    | 20         | 20         | 20         | 20         |
| Diameter I (mm)            | 38.5                       | 38.5  | 38.5       | 37.3       | 38.5       | 37.5       |
| Ho (JIS-C)                 | 59                         | 59    | 59         | 58         | 59         | 58         |
| Hs (JIS-C)                 | 86                         | 86    | 86         | 85         | 86         | 85         |
| (Hs - Ho)                  | 27                         | 27    | 27         | 27         | 27         | 27         |
| 45 <u>Mid layer</u>        |                            |       |            |            |            |            |
| Composition                | a                          | b     | d          | a          | a          | a          |
| Hm (Shore D)               | 70                         | 72    | 55         | 70         | 70         | 70         |
| Thickness (mm)             | 1.00                       | 1.00  | 1.00       | 1.00       | 1.00       | 1.00       |
| Diameter II (mm)           | 40.5                       | 40.5  | 40.5       | 39.3       | 40.5       | 39.5       |
| 50 Vm (mm <sup>3</sup> )   | 4900                       | 4900  | 4900       | 4607       | 4900       | 4655       |
| <u>Inner cover</u>         |                            |       |            |            |            |            |
| Composition                | D                          | d     | a          | d          | d          | d          |
| Hinc (Shore D)             | 55                         | 55    | 70         | 55         | 55         | 55         |
| 55 Thickness (mm)          | 0.60                       | 0.80  | 0.80       | 0.80       | 0.80       | 1.00       |
| Diameter III (mm)          | 41.7                       | 42.1  | 42.1       | 40.9       | 42.1       | 41.5       |
| Vinc (mm <sup>3</sup> )    | 3183                       | 4285  | 4285       | 4040       | 4285       | 5151       |
| <u>Outer cover</u>         |                            |       |            |            |            |            |
| Composition                | A                          | C     | A          | A          | C          | A          |
| 55 Houc (Shore D)          | 29                         | 47    | 29         | 29         | 47         | 29         |
| Thickness (mm)             | 0.50                       | 0.30  | 0.30       | 0.90       | 0.30       | 0.60       |
| Diameter IV (mm)           | 42.7                       | 42.7  | 42.7       | 42.7       | 42.7       | 42.7       |
| 60 Vouc (mm <sup>3</sup> ) | 2796                       | 1694  | 1694       | 4938       | 1694       | 3339       |

TABLE 6

| Configuration of Golf Ball |               |               |               |               |               |                |
|----------------------------|---------------|---------------|---------------|---------------|---------------|----------------|
|                            | Com.<br>Ex. 5 | Com.<br>Ex. 6 | Com.<br>Ex. 7 | Com.<br>Ex. 8 | Com.<br>Ex. 9 | Com.<br>Ex. 10 |
| <u>Core</u>                |               |               |               |               |               |                |
| Composition                | 4             | 1             | 1             | 1             | 1             | 1              |
| Vul. temp. (° C.)          | 150           | 150           | 150           | 150           | 150           | 150            |
| Vul. time (min)            | 20            | 20            | 20            | 20            | 20            | 20             |
| Diameter I (mm)            | 40.1          | 38.5          | 38.5          | 37.9          | 38.1          | 38.1           |
| Ho (JIS-C)                 | 61            | 59            | 59            | 59            | 59            | 59             |
| Hs (JIS-C)                 | 88            | 86            | 86            | 86            | 86            | 86             |
| (Hs - Ho)                  | 27            | 27            | 27            | 27            | 27            | 27             |
| <u>Mid layer</u>           |               |               |               |               |               |                |
| Composition                | a             | a             | a             | a             | a             | f              |
| Hm (Shore D)               | 70            | 70            | 70            | 70            | 70            | 62             |
| Thickness (mm)             | 1.00          | 1.60          | 1.00          | 1.30          | 0.90          | 1.00           |
| Diameter II (mm)           | 42.1          | 41.7          | 40.5          | 40.5          | 39.9          | 40.1           |
| Vm (mm³)                   | 5305          | 8087          | 4900          | 6275          | 4299          | 4802           |
| <u>Inner cover</u>         |               |               |               |               |               |                |
| Composition                | —             | —             | e             | d             | d             | d              |
| Hinc (Shore D)             | —             | —             | 43            | 55            | 55            | 55             |
| Thickness (mm)             | —             | —             | 0.8           | 0.80          | 0.80          | 0.80           |
| Diameter III (mm)          | —             | —             | 42.1          | 42.1          | 41.5          | 41.7           |
| Vine (mm³)                 | —             | —             | 4285          | 4285          | 4262          | 4203           |
| <u>Outer cover</u>         |               |               |               |               |               |                |
| Composition                | A             | C             | D             | A             | A             | B              |
| Houc (Shore D)             | 29            | 47            | 45            | 29            | 29            | 36             |
| Thickness (mm)             | 0.3           | 0.50          | 0.3           | 0.30          | 0.60          | 0.50           |
| Diameter IV (mm)           | 42.7          | 42.7          | 42.7          | 42.7          | 42.7          | 42.7           |
| Vouc (mm³)                 | 1694          | 2797          | 1694          | 1694          | 3339          | 2796           |

In Tables 4 to 6, the diameter I is the diameter (mm) of the core, the diameter II is the diameter (mm) of the sphere consisting of the core and the mid layer, the diameter III is the diameter (mm) of the sphere consisting of the core, the mid layer, and the inner cover, and the diameter IV is the diameter (mm) of the golf ball.

TABLE 7

| Results of Evaluation         |       |       |       |       |       |       |
|-------------------------------|-------|-------|-------|-------|-------|-------|
|                               | Ex. 1 | Ex. 2 | Ex. 3 | Ex. 4 | Ex. 5 | Ex. 6 |
| (Hm - Houc)                   | 41    | 41    | 34    | 43    | 41    | 36    |
| [(Vm + Vinc +<br>Vouc)/V]     | 0.27  | 0.29  | 0.27  | 0.27  | 0.27  | 0.27  |
| (Vm/Vouc)                     | 2.9   | 1.7   | 2.9   | 2.9   | 2.9   | 2.9   |
| [(Vm * Hm)/<br>(Vouc * Houc)] | 7.0   | 4.1   | 5.6   | 7.2   | 7.0   | 6.5   |
| Ratio (Vouc/V)                | 0.04  | 0.07  | 0.04  | 0.04  | 0.04  | 0.04  |
| <u>Ball characteristics</u>   |       |       |       |       |       |       |
| Db (mm)                       | 2.3   | 2.3   | 2.3   | 2.3   | 2.3   | 2.3   |
| Resilience co.                | 100   | 99    | 98    | 100   | 100   | 98    |
| (W#1)Spin (rpm)               | 2900  | 3050  | 2800  | 2800  | 3000  | 2950  |
| (W#1)Flight (m)               | 248   | 245   | 249   | 250   | 246   | 245   |
| (SW) Spin (rpm)               | 6700  | 6850  | 6550  | 6650  | 6700  | 6700  |
| Durability                    | 100   | 104   | 95    | 98    | 103   | 110   |
| Feel at impact                | A     | A     | B     | B     | B     | A     |

TABLE 8

|                               | Results of Evaluation |       |       |               |               |               |               |
|-------------------------------|-----------------------|-------|-------|---------------|---------------|---------------|---------------|
|                               | 5                     | Ex. 7 | Ex. 8 | Com.<br>Ex. 1 | Com.<br>Ex. 2 | Com.<br>Ex. 3 | Com.<br>Ex. 4 |
| (Hm - Houc)                   |                       | 41    | 25    | 26            | 41            | 23            | 41            |
| [(Vm + Vinc +<br>Vouc)/V]     |                       | 0.27  | 0.27  | 0.27          | 0.33          | 0.27          | 0.32          |
| (Vm/Vouc)                     |                       | 1.8   | 2.9   | 2.9           | 0.9           | 2.9           | 1.4           |
| [(Vm * Hm)/<br>(Vouc * Houc)] |                       | 4.2   | 4.4   | 5.5           | 2.3           | 4.3           | 3.4           |
| Ratio (Vouc/V)                |                       | 0.07  | 0.04  | 0.04          | 0.12          | 0.04          | 0.08          |
| <u>Ball characteristics</u>   |                       |       |       |               |               |               |               |
| Db (mm)                       |                       | 2.4   | 2.2   | 2.3           | 2.3           | 2.3           | 2.3           |
| Resilience co.                |                       | 99    | 98    | 99            | 92            | 96            | 94            |
| (W#1)Spin (rpm)               |                       | 3000  | 2650  | 2850          | 3200          | 2700          | 3100          |
| (W#1)Flight (m)               |                       | 246   | 253   | 250           | 240           | 250           | 242           |
| (SW) Spin (rpm)               |                       | 6850  | 6300  | 6300          | 6850          | 6300          | 6800          |
| Durability                    |                       | 103   | 84    | 65            | 105           | 85            | 103           |
| Feel at impact                |                       | A     | C     | C             | A             | C             | A             |

TABLE 9

|                               | Results of Evaluation |               |               |               |               |               |                |
|-------------------------------|-----------------------|---------------|---------------|---------------|---------------|---------------|----------------|
|                               | 25                    | Com.<br>Ex. 5 | Com.<br>Ex. 6 | Com.<br>Ex. 7 | Com.<br>Ex. 8 | Com.<br>Ex. 9 | Com.<br>Ex. 10 |
| (Hm - Houc)                   |                       | 41            | 23            | 25            | 41            | 41            | 26             |
| [(Vm + Vinc +<br>Vouc)/V]     |                       | 0.17          | 0.27          | 0.27          | 0.30          | 0.29          | 0.29           |
| (Vm/Vouc)                     |                       | 3.1           | 2.9           | 2.89          | 3.70          | 1.29          | 1.72           |
| [(Vm * Hm)/<br>(Vouc * Houc)] |                       | 7.6           | 4.3           | 4.50          | 8.94          | 3.11          | 2.96           |
| Ratio (Vouc/V)                |                       | 0.04          | 0.07          | 0.04          | 0.04          | 0.08          | 0.07           |
| <u>Ball characteristics</u>   |                       |               |               |               |               |               |                |
| Db (mm)                       |                       | 2.3           | 2.2           | 2.3           | 2.2           | 2.3           | 2.3            |
| Resilience co.                |                       | 102           | 104           | 97            | 97            | 96            | 90             |
| (W#1)Spin (rpm)               |                       | 2800          | 2700          | 2800          | 2850          | 3150          | 2900           |
| (W#1)Flight (m)               |                       | 252           | 255           | 247           | 247           | 240           | 243            |
| (SW) Spin (rpm)               |                       | 6300          | 5300          | 6000          | 6650          | 6950          | 6600           |
| Durability                    |                       | 54            | 46            | 74            | 84            | 96            | 110            |
| Feel at impact                |                       | D             | D             | D             | A             | B             |                |

As shown in Tables 7 to 9, the golf ball of each Example is excellent in all of high flight distance performance, approach performance, feel at impact, and durability. From the results of evaluation, advantages of the present invention are clear.

## INDUSTRIAL APPLICABILITY

50

The golf ball according to the present invention can be used for playing golf on golf courses and practicing at driving ranges.

## DESCRIPTION OF THE REFERENCE CHARACTERS

55

- 2 . . . golf ball
- 4 . . . core
- 6 . . . mid layer
- 8 . . . inner cover
- 10 . . . reinforcing layer
- 12 . . . outer cover
- 14 . . . dimples
- 16 . . . land

The invention claimed is:

1. A golf ball comprising a spherical core, a mid layer positioned outside the core, an inner cover positioned outside the mid layer, and an outer cover positioned outside the inner cover, wherein:

the core is obtained by a rubber composition being crosslinked, and the rubber composition includes 0.5 parts by weight or greater but less than 10 parts by weight of a fatty acid or a fatty acid metal salt per 100 parts by weight of a base rubber,

the inner cover is formed from a resin composition, a principal component of a base polymer of the resin composition is an ionomer resin, to or greater than 60% by weight,

a Shore D hardness  $H_m$  of the mid layer is greater than a Shore D hardness  $H_{inc}$  of the inner cover, and the hardness  $H_{inc}$  is greater than a Shore D hardness  $H_{ouc}$  of the outer cover,

a difference ( $H_m - H_{ouc}$ ) between the hardness  $H_m$  and the hardness  $H_{ouc}$  is greater than 25,

a volume  $V_m$  of the mid layer is greater than a volume  $V_{inc}$  of the inner cover, and the volume  $V_{inc}$  is greater than a volume  $V_{ouc}$  of the outer cover,

a ratio  $[(V_m + V_{inc} + V_{ouc})/V]$  of a sum ( $V_m + V_{inc} + V_{ouc}$ ) of the volume  $V_m$ , the volume  $V_{inc}$ , and the volume  $V_{ouc}$  relative to a volume  $V$  of an entirety of the golf ball is less than 0.30,

a ratio  $(V_m/V_{ouc})$  of the volume  $V_m$  relative to the volume  $V_{ouc}$  is greater than 1.50,

a product  $(V_m * H_m)$  of the hardness  $H_m$  and the volume  $V_m$  and a product  $(V_{ouc} * H_{ouc})$  of the hardness  $H_{ouc}$  and the volume  $V_{ouc}$  meet the following relationship:

$$[(V_m * H_m) / (V_{ouc} * H_{ouc})] > 3.0,$$

the volume  $V_{inc}$  of the inner cover is equal to or greater than  $3500 \text{ mm}^3$  but equal to or less than  $4500 \text{ mm}^3$ , and the volume  $V_{ouc}$  of the outer cover is equal to or greater than  $1500 \text{ mm}^3$  but equal to or less than  $3200 \text{ mm}^3$ .

2. The golf ball according to claim 1, wherein a ratio  $(V_{ouc}/V)$  of the volume  $V_{ouc}$  relative to the volume  $V$  is less than 0.08.

3. The golf ball according to claim 1, wherein the hardness  $H_{ouc}$  is equal to or less than 36.

4. The golf ball according to claim 1, wherein the mid layer is formed from a resin composition, and a principal component of a base resin of the resin composition is selected from an ionomer resin, a polyamide resin, and a mixture thereof.

5. The golf ball according to claim 1, wherein the hardness  $H_m$  is equal to or greater than 68.

6. The golf ball according to claim 1, wherein a JIS-C hardness  $H_s$  at a surface of the core is greater than a JIS-C hardness  $H_o$  at a central point of the core, and a difference ( $H_s - H_o$ ) between the hardness  $H_s$  and the hardness  $H_o$  is equal to or greater than 20.

7. The golf ball according to claim 1, wherein the ionomer resin is a binary copolymer formed with an  $\alpha$ -olefin and  $\alpha,\beta$ -unsaturated carboxylic acid having 3 to 8 carbon atoms.

8. The golf ball according to claim 7, wherein the core includes a base rubber selected from polybutadiene, polyisoprene, styrene-butadiene copolymer, ethylene-propylene-diene copolymer, and natural rubber.

9. The golf ball according to claim 8, wherein the polybutadiene of the core is equal to or greater than 50% by weight to the entire base rubber.

10. The golf ball according to claim 9, wherein in the polybutadiene of the core *cis*-1,4 bonds are equal to or greater than 40%.

11. The golf ball according to claim 8, wherein the core further comprises a co-crosslinking agent being a monovalent or bivalent metal salt of an  $\alpha, \beta$  unsaturated carboxylic acid having 2 to 8 carbon atoms and present at equal to or greater than 25 parts by weight and less than or equal to 45 parts by weight to the base rubber.

12. The golf ball according to claim 11, wherein the co-crosslinking agent of the core is zinc oxide and/or magnesium oxide.

13. The golf ball according to claim 11, wherein the core further comprises a fatty acid or fatty acid metal salt having a carbon number of 4 to 15 and present at equal to or greater than 1.5 parts by weight and less than or equal to 10 parts by weight to the base rubber, said fatty acid or fatty acid salt excluding the co-crosslinking agent.

14. The golf ball according to claim 13, wherein the core further comprises a filler selected from the group consisting of zinc oxide, barium sulfate, calcium carbonate, and magnesium carbonate.

15. The golf ball according to claim 14, wherein i) a JIS-C hardness  $H_o$  at the central point of the core is equal to or greater than 40 but equal to or less than 80, and ii) a JIS-C hardness  $H_s$  at the surface of the core is equal to or greater than 80 but equal to or less than 96.

16. The golf ball according to claim 15, wherein the core has an amount of compressive deformation of equal to or greater than 2.0 mm and less than or equal to 4.0 mm.

17. The golf ball according to claim 16, wherein the outer cover comprises a urethane resin or a urea resin.

\* \* \* \* \*